

## UNITED STATES PATENT OFFICE

2,331,579

## STABILIZED TEXTILE FINISH

Harold W. Stiegler, Stamford, and John M. Hood, Riverside, Conn., assignors to American Cyanamid Company, New York, N. Y., a corporation of Maine

No Drawing. Application March 7, 1942,  
Serial No. 433,788

8 Claims. (Cl. 252—8.7)

This invention relates to the finishing of textiles and more particularly to the softening of textiles such as threads and filaments, woven cloth and the like by the impregnation or coating thereof with stabilized unsulfonated or sulfonated glyceride oils and fats, waxes and mineral oils, and with mixtures containing any one or more of these softening agents. The invention includes the stabilized softening agents themselves, their methods of preparation, and softened textiles impregnated or coated therewith.

In the finishing of textiles such as plain or dyed threads or fabrics composed of cotton, linen, wool, silk and the like, it is customary to apply a softening agent in the form of a solution or aqueous emulsion. The softening agents now most commonly employed for these purposes almost always contain greater or lesser amounts of unsulfonated or sulfonated glycerides of higher fatty acids or completely or partially emulsifiable waxes such as japan wax, beeswax, carnauba wax, scale wax and the like, and such softening agents have frequently caused trouble by oxidation and rancidity. Such oxidation is particularly troublesome when it occurs after the softener has been applied to a dyed fabric, for it causes fading of the dyes.

Our present invention is based on the discovery that the oxidation and rancidity of textile finishing and softening agents containing unsulfonated or sulfonated higher fatty acid glycerides or waxes of the type now in commercial use can be avoided by the incorporation therein of small but effective amounts of a metal bisulfite-formaldehyde addition compound. We have found that a stabilizer of this class is effective to prevent auto-oxidation and rancidity in either unsulfonated or sulfonated glyceride oils and fats and waxes even when these substances are exposed to the atmosphere in finely divided condition, as is the case when they have been applied as a finish to textiles.

While the fats and waxes for textile use may be stabilized with the addition compound of any metal bisulfite and formaldehyde better results may be had by employing those obtainable by reacting an alkali metal bisulfite with formaldehyde. This is true because the alkali metals form soluble soaps with the fatty acids, whereas certain of the other metals will form insoluble soaps therewith which if deposited in the fabric would cause guminess and spotting, and in the case of the colored insoluble soaps, such as would be formed with iron, discoloration of the fabric also.

An example of the alkali metal bisulfite-formaldehyde addition compounds, and preferred from the standpoint of cost and availability, is sodium bisulfite-formaldehyde.

The addition compounds constituting stabilizers of the present invention may be prepared by reacting a metal bisulfite with formaldehyde. Their preparation is exemplified by the preparation of sodium bisulfite-formaldehyde. 10 parts by weight of sodium bisulfite are slowly added with stirring to 8 parts by weight of 38% formaldehyde. The mixture becomes warm and may be cooled if too much heat is developed. The product is a thick white paste containing about 70-72% of sodium bisulfite-formaldehyde. The product so prepared may be used either in paste or powder form, and in the latter case water is added to the material to be stabilized at least in amounts sufficient to dissolve the powder.

20 The amount of the stabilizing compound to be added to the fat or wax will, in general, be comprised within the limits of about 1% to 6% by weight on the fat or wax, the latter being taken on the moisture-free basis. The amounts here given are not, however, to be construed as a limitation on the invention since the use of larger amounts for the purpose is contemplated and is within the scope of the invention.

25 The addition compound may be incorporated in the fat or wax when the latter is in the concentrated or manufactured state, or it may be admixed with emulsions or solutions of the materials such as are prepared for application to textiles.

30 Although they may be incorporated in any suitable manner, a preferred method is to stir a small quantity of the stabilizer in paste form with the fat or wax in fluid condition. In the case of the normally solid fats and waxes, these may be warmed slightly to obtain a partially fluid condition before incorporating the stabilizer.

35 The fats and waxes which have been partially or completely protected or stabilized may be used in admixture with each other or with unstabilized oils, fats and waxes or with mineral oils and in the form of emulsions or solutions or they may be employed with other textile finishing or treating agents such as the soluble starches, soluble gums, gluings and the like.

40 45 50 55 In the following examples, which are intended as illustrative of the invention and not as limitation thereof, sodium bisulfite-formaldehyde was used to stabilize the materials. The parts are by weight calculated on the moisture-free weight of the materials unless otherwise noted.

*Example 1*

Samples of cotton cloth were impregnated with a 5% emulsion of sulfonated tallow. Other samples were impregnated with a 5% emulsion of sulfonated tallow which had been intimately mixed with 5% of sodium bisulfite-formaldehyde. All the samples were dried.

One set of these samples together with a blank (untreated cotton cloth) was steamed for 45 minutes at 15 pounds pressure. The other set was exposed for 26 hours to dry heat (100° C.) in circulating air. All the samples were analyzed in a spectrophotometer for reflectance at 4000 Angstrom units before and after the steam and heat tests. The percent discoloration was recorded as follows:

|                                                  | Steaming test | Dry heat test |
|--------------------------------------------------|---------------|---------------|
| Blank                                            |               |               |
| Sulfonated tallow                                | 4.7           | 7.5           |
| Sulfonated tallow plus 4% bisulfite-formaldehyde | 8.9           | 19.0          |
|                                                  | 5.0           | 8.7           |

From these results it is seen that the bisulfite-formaldehyde remarkably improved the resistance of the sulfonated tallow to discoloration both by steaming and by dry heat. A further analysis of the above results shows that, after steaming, the cotton cloth treated with the sulfonated tallow containing bisulfite-formaldehyde was about 44% less discolored than the cloth treated with the sulfonated tallow alone. Where dry heat was applied to the cloth samples, 54% less discoloration was obtained over the non-stabilized sulfonated tallow.

Rancidity tests were conducted on samples of cloth impregnated respectively with the sulfonated tallow and the sulfonated tallow containing 4% sodium bisulfite-formaldehyde. The samples were stored in sealed glass jars at 50° C. with the result that while the sulfonated tallow alone became rancid in two weeks that containing the sodium bisulfite-formaldehyde showed no rancidity at the end of a month. In this respect similar tests carried out with another type of sulfonated tallow showed the sulfonated tallow alone to become rancid after 217 hours whereas the one containing the sodium bisulfite-formaldehyde was not rancid after 624 hours.

Samples of cotton cloth were sized respectively with the sulfonated tallow containing and not containing sodium bisulfite-formaldehyde and stored exposed to the air for two weeks and then steamed at 15 pounds pressure. The bisulfite-formaldehyde protected sample gave a better white than the control. Further samples of the cloth were then examined after storage for six months. The samples sized with the stabilized sulfonated tallow were whiter than those containing the unprotected sulfonated tallow. Portions of these samples were then subjected to the steaming test and it was found that the bisulfite-formaldehyde had retained its effectiveness and gave a better white than the non-stabilized sulfonated tallow.

Any of the tallows now known to the textile trade as finishes, whether of animal or vegetable origin, may be stabilized in accordance with the invention and therefore the term "sulfonated tallow" as used in the claims is intended to include such tallows. The term "higher fatty acid glyceride" is used to define the glycerides of saturated and unsaturated fatty acids of 8

or more carbon atoms such as are found in fats and oils of animal and vegetable origin.

*Example 2*

Tests similar to those of Example 1 were conducted on a fabric softener which consisted of japan wax and beeswax emulsified with sodium hydroxide, stearic acid and water. In these tests samples of unfinished bleached cotton cloth were impregnated in each case with 5% emulsions of the softener, one emulsion being used for the control and containing no stabilizer, whereas the saponified waxes of the other emulsions contained 2.5% and 5%, respectively, of sodium bisulfite-formaldehyde. The samples were then dried and submitted to three types of severe ageing tests. These tests consisted in (1) subjecting samples to a 3/4 hour steaming at 15 pounds pressure and a temperature of 250° F.; (2) exposing samples in a current of air for five hours at a temperature of 250° F.; and (3) sealing cloth samples in glass jars for 5 hours at a temperature of 250° F.

These tests showed the control to be yellow whereas the samples containing the bisulfite-formaldehyde were of improved color. The sample treated with the softener to which the higher percentage of the stabilizing agent had been added showed a clear bright white.

It is to be understood that the invention is not limited to the stabilization of the emulsifiable waxes, japan and beeswax, given in Example 2, but may be extended to other emulsifiable waxes, whether of animal, vegetable or of mineral origin, such as, scale wax, carnauba wax, montan wax, ceresin wax, candelilla wax. Briefly, then, the metal bisulfite-formaldehyde compounds, and more particularly the alkali metal bisulfite-formaldehyde compounds, may be employed to partially or completely protect or stabilize any of the emulsifiable waxes which tend to become discolored or rancid.

*Example 3*

45 Indigo dyed light blue denim cloth was finished in the usual manner by impregnation with aqueous dispersions containing 0.5 lb. per gallon of the following sulfonated vegetable and animal oils and fats.

50 75% sulfonated tallow plus 25% unsulfonated tallow

Incompletely sulfonated castor oil

Sulfonated mixture of equal parts of peanut oil, coconut oil and white olein

55 Mixture of equal parts of sulfonated peanut oil, sulfonated white olein, and mineral oil

All the impregnated samples faded considerably when they were subjected to the heating and oxidation tests described in Example 1.

60 26.3 pounds of sodium bisulfite were dissolved in 52.6 pounds of water and 21 pounds of 37% aqueous formaldehyde solution were slowly added with stirring. Sufficient of the resulting sodium bisulfite-formaldehyde was added to each of the above dispersions to make 0.125 pounds per gallon on the dry weight of the stabilizer and additional samples of the cloth were impregnated therewith, dried, and subjected to the heating and oxidation tests. It was found that fading was almost completely absent.

This is a continuation-in-part of our copending application, Serial No. 351,104, filed August 3, 1940.

What we claim is:

1. A textile finishing composition comprising

a member of the group consisting of higher fatty acid glycerides and sulfonated higher fatty acid glycerides together with stabilizing amounts of a metal bisulfite-formaldehyde addition compound.

2. A textile finishing composition comprising a sulfonated glyceride oil together with stabilizing amounts of a metal bisulfite-formaldehyde addition compound.

3. A textile finishing composition comprising a member of the group consisting of higher fatty acid glycerides and sulfonated higher fatty acid glycerides together with stabilizing amounts of an alkali metal bisulfite-formaldehyde addition compound.

4. A textile finishing composition comprising a sulfonated glyceride oil together with stabilizing amounts of an alkali metal bisulfite-formaldehyde addition compound.

5. Textile material impregnated with at least 20 one of the textile finishes of the group consisting

of emulsifiable waxes and sulfonated fats having incorporated therein stabilizing amounts of an alkali-metal bisulfite-formaldehyde addition compound.

5. 6. Textile material impregnated with at least one of the textile finishes of the group consisting of emulsifiable waxes and sulfonated fats having incorporated therein stabilizing amounts of sodium bisulfite-formaldehyde addition compound.

7. Textile material impregnated with a sulfonated tallow having incorporated therein stabilizing amounts of sodium bisulfite-formaldehyde addition compound.

15 8. Textile material impregnated with wax having incorporated therein stabilizing amounts of sodium bisulfite-formaldehyde addition compound.

HAROLD W. STIEGLER.  
JOHN M. HOOD.